

1

3,728,122  
ONE-COMPONENT DIAZOTYPE LIGHT-  
SENSITIVE MATERIAL

Shigeaki Yoshida, Yokohama, Shuhei Shiraishi, Fujisawa, and Fumio Yuki, Tokyo, Japan, assignors to Ricoh Co., Ltd., Tokyo, Japan  
No Drawing. Filed Dec. 16, 1970, Ser. No. 98,932  
Claims priority, application Japan, Dec. 17, 1969,  
44/100,878  
Int. Cl. G03c 1/60

U.S. Cl. 96—75

5 Claims

ABSTRACT OF THE DISCLOSURE

One-component diazotype light-sensitive material containing a condensation product made from naphthalene-sulfonate or alkynaphthalenesulfonate and formaldehyde as a stabilizer in a precoat layer on a supporting sheet, said material having good stability.

BACKGROUND OF THE INVENTION

One-component diazotype light-sensitive material commonly comprises a supporting sheet having, on a surface thereof, a light-sensitive layer containing a stabilized light-sensitive diazonium compound which couples with an azo coupling component in an alkaline medium to form a visible azo dyestuff. Diazonium compounds as a general rule are not stable at higher temperatures. Normally those compounds having the highest sensitivity have the lowest stability with increasing temperature and humidity. Thus, the diazonium compounds having the better sensitivity because they react readily with the azo coupling component most readily decompose at higher temperatures and humidity. Acid stabilizers are often employed to alleviate this difficulty.

Diazotype light-sensitive materials disclosed in British Pat. 867,630 and Japanese patent publication 6,233/1961, include highly sensitive diazonium compounds having the following general formula:



in which X is an acid anion, Y is a fluorine or chlorine atom, R<sub>4</sub> and R<sub>5</sub> are chosen from alkyl, hydroxyalkyl and chloralkyl groups having at most 4 carbon atoms and aralkyl groups and nuclear substituted chloroaralkyl groups having at most 11 carbon atoms, R<sub>6</sub> is chosen from alkyl groups having at most 4 carbon atoms and aralkyl groups having at most 11 carbon atoms, and R<sub>4</sub>, R<sub>5</sub>, and R<sub>6</sub> contain together at least 6 and at most 17 carbon atoms.

In the above-mentioned diazotype light-sensitive material, organic acids such as citric acid or tartaric acid or inorganic acids such as boric acid or sulfuric acid are often used as acid stabilizers. The foregoing diazonium compounds decompose at temperatures as low as 80° C. to 100° C. They decompose slowly during the summer even when they are stabilized by acid. This causes an "autocoupling" with the decomposition products which is manifested by the fogging of the light-sensitive material. Consequently, light-sensitive material containing highly sensitive diazonium compounds such as those mentioned above cannot be preserved for a long time and have a relatively short shelf life.

Various proposals have been made to eliminate this defect. For example, in Japanese patent publication 17,238/1963, the use of salts of alkali metals of naphthalene mono-, -di- or -tri-sulfonic acid as stabilizers is suggested.

2

This solution to the problem has not proved to be satisfactory since these salts and the above mentioned diazonium compounds interact and coagulate to form a tar-like material.

In order to diminish this coagulation and the formation of the tar-like products, it has been proposed to form a precoat layer containing such stabilizers, together with starch or silica on a support, and then to apply an aqueous light-sensitive solution containing the diazonium compound to the precoat layer. Even when this method is used, however, the stabilizer dissolves into the light-sensitive solution being applied to the substrate and reacts with the diazonium compound to form the tar-like products. A light-sensitive material prepared under such conditions cannot yield a good dye-image with a clear background and does not have good stability.

It is, therefore, an object of the present invention to alleviate the above-mentioned disadvantage and to provide a stable one-component diazotype light-sensitive material.

THE INVENTION

The present invention relates to a one-component diazotype light-sensitive material having high preservability which contains a condensation product made from naphthalenesulfonate or alkynaphthalenesulfonate and formaldehyde in a precoat layer on a surface of a supporting sheet.

The condensation products used in this invention have the following general formula:



wherein R<sub>1</sub>, R<sub>2</sub> and R<sub>3</sub> are hydrogen or alkyl containing from about 1 to 5 carbon atoms, X is sodium or potassium, and n is from about 0 to 8.

These condensation products are known as anion surface active agents. It has now been discovered that they are effective to improve the stability of diazonium compounds. Since these stabilizing agents have sulfonic acid groups which would interact with the diazonium compounds, they cannot be used by dissolving them together with the diazonium compound in a light-sensitive solution. Satisfactory results can be obtained however by using them dispersed in a precoat layer comprising starch, powdered silica, polyvinyl acetate or like excipients.

A typical precoat composition for forming the precoat layer would contain, for example, 100 g. of fine powdered cornstarch, 20 g. of fine powdered silica and 95 g. of polyvinyl acetate emulsion having a 50% solids content in 1000 cc. of water, together with 1 g. to 10 g. of the stabilizer.

The compositions most useful in the practice of this invention are those in which the amount of stabilizer used is from about 0.1 to 1.0 gram per gram of diazonium compound. The composition may be spread on the support sheet by any convenient method, for example, roller coating. As spread it will normally be of a thickness such that the coat will contain from about 0.01 to 0.15 gram of stabilizer per square meter of support sheet. Appreciable variations from these ranges can be tolerated while still obtaining useful results.

The preparation of the condensation products utilized in this invention follows standard procedures. It is normally not practical to prepare and isolate pure compounds. Fortunately, it is not necessary to use pure compounds in the practice of the invention. The mixtures obtained by the usual synthetic techniques can be employed. Those

products in which the mean value of  $n$  is from about 0 to 8 are preferably used.

Typical stabilizing condensation products which may be used in the practice of this invention include the following in which  $n$  has the same meaning as above.

(1) Condensation product made from sodium naphthalenesulfonate and formaldehyde:



(2) Condensation product (Compound B) made from sodium methylnaphthalenesulfonate and formaldehyde;



(3) Condensation product (Compound C) made from sodium propylnaphthalenesulfonate and formaldehyde;



(4) Condensation product (Compound D) made from sodium butylnaphthalenesulfonate and formaldehyde;



(5) Condensation product (Compound E) made from sodium amylnaphthalenesulfonate and formaldehyde;



(6) Condensation product (Compound F) made from sodium naphthalenesulfonate, sodium butylnaphthalenesulfonate and formaldehyde;



(7) Condensation product (Compounds G and H) made from sodium propylnaphthalenesulfonate, sodium butylnaphthalenesulfonate and formaldehyde;



20 Similar products are obtained from other naphthalenesulfonates in which the sodium is replaced with potassium and the alkyl group is on a portion other than the 4-position on the naphthalene nucleus.

The following non-limiting examples are given by way 25 of illustration only.

#### EXAMPLE 1

A precoat mixture was prepared from the following 30 ingredients:

|                                             |    |      |
|---------------------------------------------|----|------|
| Water                                       | cc | 1000 |
| Cornstarch (particle size: 1-5 $\mu$ )      | g  | 100  |
| Powdered silica (particle size: 1-5 $\mu$ ) | g  | 20   |
| 35 Polyvinyl acetate emulsion (solid: 50%)  | g  | 95   |
| Compound A; $n \approx 2-4$                 | g  | 3    |

A light-sensitive solution (a solution for forming a 40 light-sensitive layer) was prepared from the following ingredients:

|                                                                                            |    |      |
|--------------------------------------------------------------------------------------------|----|------|
| Water                                                                                      | cc | 1000 |
| Tartaric acid                                                                              | g  | 10   |
| 45 Concentrated sulfuric acid                                                              | cc | 4    |
| 2 - phenoxy - 5 - chloro - 4 - dibenzylaminobenzene diazonium chloride $\frac{1}{2}ZnCl_2$ | g  | 9.5  |
| Methylene blue                                                                             | g  | 0.1  |
| Saponin                                                                                    | g  | 1    |

50 The precoat composition was applied to a surface of a supporting sheet and dried off and then the light-sensitive solution was applied to the surface and dried off to provide a one-component diazotype light-sensitive material 55 (Sample A). Another light-sensitive material (Sample B) for comparative test was obtained by repeating the same procedure except that the precoat composition did not contain Compound A. Sample A' and Sample B' were 60 prepared by subjecting Samples A and B to artificial aging by keeping them in a desiccator at a temperature of 50° C. and a relative humidity (RH) of 50% for 48 hours. The comparative test of Samples A, A', B and B' was carried out as follows:

65 A black dye-image was formed on each sample by overlaying an image-carrying original on each sample, exposing it to light and then developing it in the following liquid developer:

|                    |    |      |
|--------------------|----|------|
| 70 Water           | cc | 1000 |
| Thiourea           | g  | 10   |
| Phloroglucin       | g  | 5    |
| Citric acid        | g  | 1    |
| Sodium citrate     | g  | 80   |
| 75 Sodium benzoate | g  | 20   |

Densities of the dye-images and the backgrounds (non-image area of the sample) were measured to compare and the following results were obtained.

|                       | Density of— |            |
|-----------------------|-------------|------------|
|                       | Dye-image   | Background |
| <b>Sample:</b>        |             |            |
| A                     | 1.12        | 0.12       |
| A'                    | 1.10        | 0.13       |
| Difference of density | -0.02       | +0.01      |
| <b>Sample:</b>        |             |            |
| B                     | 1.11        | 0.12       |
| B'                    | 0.58        | 0.21       |
| Difference of density | -0.53       | +0.09      |

The density was measured with a "Photovolt densitometer," sold by "Photovolt Co.," using a green filter.

From these results, the advantageous stabilizing action effect of the condensation product made from sodium naphthalenesulfonate and formaldehyde can be detected.

#### EXAMPLE 2

One-component diazotype light-sensitive materials were obtained by repeating the same procedure as that of Example 1 except that the aforementioned Compound F ( $n \approx 2$ ) was employed instead of Compound A in the precoat solution and the comparative test was carried out in the same manner as that of Example 1. The results thus obtained were similar to that of Example 1.

Compound F ( $n \approx 2$ ) used in this example was made as follows:

Butylnaphthalenesulfonic acid was obtained by the condensation of 30 cc. of butyl alcohol and 80 g. of naphthalene in the presence of 35 cc. of concentrated sulfuric acid. 30 g. of butylnaphthalenesulfonic acid and 5 g. of powdered naphthalene were mixed in a mixture of 40 g. of concentrated sulfuric acid and 10 cc. of water, and then 11 cc. of 30% aqueous solution of formaldehyde were added to the mixture under stirring at a temperature between 50° C. and 60° C. and the stirring was continued at this temperature for 3.5 hours to separate the reaction product as a viscous mass. The desired condensation product, Compound F (18 g.) was obtained by the neutralization of this viscous mass with sodium hydroxide.

#### EXAMPLE 3

One-component diazotype light-sensitive materials were obtained by repeating the same procedure as that of Example 1 except that the aforementioned Compound D ( $n \approx 1.4$ ) was employed instead of Compound A in the precoat solution, and the comparative test was carried out in the same manner as that of Example 1. The results thus obtained were similar to that of Example 1.

Compound D ( $n \approx 1.4$ ) used in this example was made as follows:

After 6 g. of powdered naphthalene were added to dibutyl sulfate made from 25 cc. of concentrated sulfuric acid and 7 cc. of n-butyl alcohol, this mixture was stirred for a while at a temperature of 50° C. As cooled, the mixture separated into two layers. The lower layer was removed and 5 cc. of 30% aqueous solution of formaldehyde were added to the upper layer (butylnaphthalenesulfonic acid) under stirring at a temperature of 50° C. and the stirring was continued at a temperature between 50° C. and 60° C. until the reaction was complete, as indicated by the disappearance of formaldehyde. After cooling, the mixture separated into two (upper and lower) layers. The desired condensation product, Compound D (4.5 g.), was obtained by the neutralization of the reaction product of the upper layer with sodium hydroxide.

#### EXAMPLE 4

A precoat composition was prepared from the following ingredients:

|   |                                         |    |      |
|---|-----------------------------------------|----|------|
| 5 | Water                                   | cc | 1000 |
|   | Colloidal silica                        | g  | 20   |
|   | Polyvinyl acetate emulsion (solid: 50%) | g  | 40   |
|   | Compound D ( $n \approx 1.4$ )          | g  | 5    |

10 A light-sensitive solution was prepared from the following ingredients:

|    |                                                                                            |    |      |
|----|--------------------------------------------------------------------------------------------|----|------|
| 10 | Water                                                                                      | cc | 1000 |
|    | Tartaric acid                                                                              | g  | 10   |
|    | Concentrated sulfuric acid                                                                 | cc | 4    |
| 15 | 2 - methoxy - 5 - chloro-4-methylbenzylaminobenzene diazonium chloride $\frac{1}{2}ZnCl_2$ | g  | 10   |
|    | Methylene blue                                                                             | g  | 0.1  |
|    | Saponin                                                                                    | g  | 1    |

20 Two kinds of one-component diazotype light-sensitive materials with or without Compound D, i.e. Sample A<sub>1</sub> and B<sub>1</sub>, were prepared in the same procedure as that of Example 1 except that the above-mentioned precoat solution with or without Compound D and the light-sensitive solution prepared above were used, and then they were 25 subjected to artificial aging as described in Example 1.

Samples A<sub>1</sub>' and B<sub>1</sub>' thus aged were treated and developed in the same manner as that of Example 1 except that the following liquid developer, and black dye-images formed on each sample (A<sub>1</sub>' and B<sub>1</sub>') were compared.

#### 30 Liquid developer:

|    |                 |    |      |
|----|-----------------|----|------|
| 30 | Water           | cc | 1000 |
|    | Thiourea        | g  | 15   |
|    | Phloroglucin    | g  | 4    |
| 35 | Benzoic acid    | g  | 25   |
|    | Sodium benzoate | g  | 15   |
|    | Sodium formate  | g  | 150  |

40 Sample A<sub>1</sub>' gave a clear, black dye-image having good intensity on the vivid background, while Sample B<sub>1</sub>' gave an unclear dye-image of very low density.

#### EXAMPLE 5

One-component diazotype light-sensitive materials were obtained by repeating the same procedure as that 45 of Example 4 except that 4 g. of the aforementioned Compound G ( $n \approx 5$ ) was employed instead of 5 g. of Compound D ( $n \approx 1.4$ ) in the precoat solution, and the comparative test was carried out in the same manner as that of Example 4. The results thus obtained were similar 50 to that of Example 4.

Compound G ( $n \approx 5$ ) used in this example was made as follows:

55 Butylnaphthalenesulfonic acid was obtained by the condensation of 12 cc. of butyl alcohol and 15 g. of naphthalene in 20 cc. of concentrated sulfuric acid, and propylnaphthalenesulfonic acid was obtained by the condensation of 25 cc. of propyl alcohol and 30 g. of naphthalene in 37 cc. of concentrated sulfuric acid. 32 g. of butylnaphthalenesulfonic acid and 30 g. of propylnaphthalenesulfonic acid were mixed in 70 cc. of concentrated sulfuric acid, and then 11 cc. of 30% aqueous solution of formaldehyde were added to the mixture under stirring at a temperature between 50° C. and 60° C. and the stirring was continued for about 8 hours while 60 slowly raising the temperature to 100° C. at last. As allowed to stand, the mixture separated into two layers. The desired Compound G (19 g.) was obtained by the neutralization of the reaction product of the upper layer with sodium hydroxide.

70 What is claimed is:

1. One-component diazotype light-sensitive material comprising a precoat layer between a supporting sheet and a light-sensitive layer containing a diazonium compound, the precoat layer containing from about 0.01 to 75 0.15 gram per square meter of support sheet of a stabiliz-

7  
ing compound having the following formula dispersed in an excipient:



wherein

R<sub>1</sub>, R<sub>2</sub> and R<sub>3</sub> are hydrogen or alkyl containing from about 1 to 5 carbon atoms,  
X is sodium or potassium, and  
n is an integer from about 0 to 8.

2. A light-sensitive material as in claim 1 wherein the stabilizing compound is represented by the formula:



3. A light-sensitive material as in claim 1 wherein the stabilizing compound is represented by the formula:



4. A light-sensitive material as in claim 1 wherein the stabilizing compound is represented by the formula:



5. A light-sensitive material as in claim 1 wherein the stabilizing compound is represented by the formula:



10

#### References Cited

#### UNITED STATES PATENTS

|           |         |                   |       |         |
|-----------|---------|-------------------|-------|---------|
| 3,102,812 | 9/1963  | Welch             | ----- | 96-91 R |
| 2,498,722 | 2/1950  | Straley           | ----- | 96-91 R |
| 2,807,545 | 9/1957  | Frederick         | ----- | 96-91 R |
| 3,153,592 | 10/1964 | Klimkowski et al. | ----- | 96-91 R |
| 2,541,727 | 2/1951  | Von Glahn et al.  | ----- | 96-91 R |
| 2,545,423 | 3/1951  | Duerr             | ----- | 96-91 R |
| 2,593,911 | 4/1952  | Neumann et al.    | ----- | 96-91 R |

#### FOREIGN PATENTS

|         |        |               |       |         |
|---------|--------|---------------|-------|---------|
| 571,802 | 9/1945 | Great Britain | ----- | 96-91 R |
| 609,912 | 3/1962 | Belgium       | ----- | 96-49   |

#### OTHER REFERENCES

- Dinaburg, M. S., "Photosensitive Diazo Compounds," The Focal Press, 1964, p. 93 relied on.  
30 Muller, P., "Precoat of Diazoype Paper," Tappi, August 1965, pp. 55A-59A.

CHARLES L. BOWERS, JR., Primary Examiner

35 U.S. CL. X.R.  
96-49, 91 R

40